

# United States Patent [19]

Stevens et al.

[11] 3,867,213

[45] Feb. 18, 1975

[54] **FERROCENE-CONTAINING MONOMERS AND COPOLYMERS**

[75] Inventors: **Trevis E. Stevens; Samuel F. Reed, Jr.**, both of Huntsville, Ala.

[73] Assignee: **The United States of America as represented by the Secretary of the Army**, Washington, D.C.

[22] Filed: **May 18, 1971**

[21] Appl. No.: **144,280**

**Related U.S. Application Data**

[62] Division of Ser. No. 849,254, July 31, 1969.

[52] U.S. Cl..... **149/19.2, 149/19.5, 149/19.1, 149/19.91, 149/20**

[51] Int. Cl..... **C06d 5/06**

[58] Field of Search .... **149/19.2, 19.9, 19.5, 19.91, 149/20**

[56] **References Cited**

UNITED STATES PATENTS

|           |         |                    |          |
|-----------|---------|--------------------|----------|
| 3,718,633 | 2/1973  | Baldwin .....      | 149/19.2 |
| 3,739,004 | 6/1973  | Ponder et al. .... | 149/19.2 |
| 3,770,787 | 11/1973 | Burnett.....       | 149/19.2 |

**OTHER PUBLICATIONS**

Pittman et al., *Macromolecules*, Vol. 3, (1970), pp. 746-754 [QD380M3].

Neuse, *Ferrocene Polymers, Advances in Macromolecular Chemistry*, Ed. by W. M. Pasika, Vol. I, Academic Press, N.Y., (1968) pp. 1-28 [QD380A2].

*Primary Examiner*—Benjamin R. Padgett  
*Attorney, Agent, or Firm*—Edward J. Kelly; Herbert Berl; Jack W. Voigt

[57] **ABSTRACT**

The ferrocene-containing polymerizable monomers, pentaerythritol methacrylate tris (ferrocenoate) and pentaerythritol acrylate tris (ferrocenoate), are disclosed along with the pertinent preparative procedures therefor. The specified ferrocene-containing monomers when copolymerized with butadiene serve as the propellant binder and catalyst for fast-burning composite propellants. The copolymers perform the functions of binder and catalyst in a propellant composition containing ammonium perchlorate, a plasticizer, and aluminum metal fuel.

**2 Claims, No Drawings**

## FERROCENE-CONTAINING MONOMERS AND COPOLYMERS

Cross-Reference to Related Application:

This is a division of application Ser. No. 849,254, filed July 31, 1969.

### BACKGROUND OF THE INVENTION

Prior art compounds resulting from the selective partial esterification of pentaerythritol are known. Two derivatives of pentaerythritol which serve as the starting compounds for the preparation of the ferrocene containing monomers of this invention are pentaerythritol arsenite methacrylate and pentaerythritol arsenite acrylate.

The term polymerizable monomer is well known. The term when applied to the propellant art generally means a compound useful in propellants because it is capable of forming an elastic tough rubbery polymer by condensation or polymerization reactions in the propellant mix. The resulting rubbery polymer functions as a binder for the propellant charge. The binder provides strength for the propellant charge or grain. Many of the prior art compounds have been concerned with binder materials. The present trend has been to increase the performance of propellants by employing an energetic binder material, improved oxidizer, and burning rate catalyst.

The prior art esters of polymerizable compounds have been employed as energetic binder materials having oxidizing and plasticizing capabilities. The term energetic binder is a term to distinguish one type of binder from another type of binder known as non-energetic binder. The non-energetic binders provide binding functions while contributing little, if any, to the propellant burning processes. The propellant burning process is a complex process requiring a proper balance of fuel, oxidizer, and catalysts. The oxygen content of a number of energetic binders of the prior art enables those binders to contribute to the oxidizing capability of the propellant composition in addition to the binding capability of the propellant composition. Each active ingredient in a propellant composition contributes to one or more functions of the propellant system. Naturally, a multi-functional ingredient offers distinct advantages.

Generally, a burning rate additive has been required for use in the prior art propellant compositions to obtain increased burning rates. These additives or catalysts have included metallic oxides and organo-metallic compounds. Ferrocene and n-butyl ferrocene have been utilized as burning rate catalysts. The liquid ferrocene compounds have been effective in promoting burning rates. However, like all liquids used as additives, the characteristic disadvantages of liquid additives such as loss by evaporation, migration, etc., have caused processing problems as well as problems encountered later during long term storage of propellants.

An additive which is not subject to the disadvantages of some of the prior art compounds would be attractive for use in propellants.

The present invention has as its principal object to provide ferrocene-containing monomers which can be polymerized to form an energetic binder having a burning rate catalyst as an integral part thereof.

Another object is to provide copolymerization products of ferrocene-containing monomers and butadiene

which serves as energetic binder and burning rate catalyst for propellant compositions.

A further object of this invention is to provide a propellant composition having a combination energetic binder and catalyst which does not evaporate during propellant processing or migrate in the finished propellant.

Summary of the Invention: The ferrocene-containing monomers, pentaerythritol methacrylate tris (ferrocenoate) and pentaerythritol acrylate tris (ferrocenoate) are produced from pentaerythritol arsenite methacrylate and pentaerythritol arsenite acrylate respectively as the starting compounds. The monomers become constituents of copolymers of butadiene when polymerization reaction is initiated by a suitable initiator. The copolymers of this invention are useful as binders for solid propellants which also contain an oxidizer, metal fuel, and plasticizer. The binders also function as a burning rate catalyst since the catalyst is an integral part thereof. The catalyst being an integral part of the cured binder does not migrate during propellant storage. The catalyst is evenly and widely dispersed as an integral part of the binder; therefore, this arrangement is conducive to uniform burning rate control and stability to burning of the propellant composition.

Description of the Preferred Embodiments: The starting compound, pentaerythritol arsenite methacrylate, forms one of the monomers of this invention and may be produced as follows:

30 To a clear solution of 10.4 grams (0.050 mole) of pentaerythritol arsenite in 20 milliliters of acetonitrile and 8 milliliters of triethylamine is added drop wise a mixture of 5.5g. (0.052 mole) of methacryloyl chloride and 5 ml. of acetonitrile. The addition requires about 35 15 minutes while the temperature is maintained at about 35°C to about 40°C by external cooling. The mixture is stirred at 50°C for 2 hours, then the solvent is removed at reduced pressure, and the residue is dried at ambient temperature and 1 millimeter of pressure for 40 30 minutes. The residue is extracted with three 100 ml. portions of hot ligroin (each containing 5 mg. of hydroquinone). The extracts are concentrated and chilled and the product removed by filtration. The solid obtained is recrystallized from ligroin to give 5.40 grams of the monomer, pentaerythritol arsenite methacrylate, m.p. 83°C to 84.5°C.

Another starting compound, pentaerythritol arsenite acrylate, forms another monomer and may be produced as follows:

50 To a mixture of 10.4g. (0.050 mole) of pentaerythritol arsenite and 10 ml. of acetonitrile is added 4.5 ml. (0.065 mole) of acrylic acid followed by 24 ml. (0.175 mole) of triethylamine. When the exotherm from the addition of the amine (the reaction temperature should not be allowed to exceed 20°C) is subsided, 7.7 ml (0.060 mole) of benzene-sulfonyl chloride in 10 ml. of acetonitrile is added over a 15 minute period. The reaction mixture is cooled to keep the temperature below 55 30°C during the addition; after the benzenesulfonyl chloride addition, the mixture is stirred at 30°C for one hour. The solvent is then removed at reduced pressure and the residue dried at ambient temperature and 1 millimeter of pressure for 30 minutes. The residue is extracted three times with 200 ml. of hot ligroin containing 0.01g of hydroquinone. The residue is taken up in methylene chloride and again stripped to dryness. Recrystallization from ligroin yields the monomer, pen-

taerythritol arsenite acrylate, 7.4g. m.p. 80°C to 82°C.

Pentaerythritol methacrylate tris (ferrocenoate) and pentaerythritol acrylate tris (ferrocenoate) are mono-

vents is re-crystallized from methanol. The yield is pentaerythritol acrylate tris (ferrocenoate), 1.05 g, m.p. 107°-109°C.

Analysis

Calculated for  $C_{41}H_{38}Fe_3O_8$ : C, 59.60; H, 4.64; Fe, 20.3.

Found: C, 59.1; H, 4.59; Fe, 19.7.

mers which are prepared as set forth hereinbelow under Examples I and II. The specified monomers when copolymerized with butadiene form binders that provide in addition to the binder function the function of catalysis for the propellant system wherein used. Example III and Example IV are illustrative of the procedures for preparation of the copolymers of this invention. Table I sets forth burning rates of uncured composite propellants using the hydroxy-terminated copolymer of butadiene and pentaerythritol methacrylate tris (ferrocenoate) as compared with a propellant using unmodified hydroxy-terminated polybutadiene, and a propellant using n-butyl ferrocene, a standard burning-rate promoter. Similarly, the copolymer of pentaerythritol acrylate tris (ferrocenoate) and butadiene may be used as the binder and catalyst for a propellant composition.

**EXAMPLE I**

**Preparation of Pentaerythritol Methacrylate Tris (ferrocenoate)**

A 2.20 g. (8 mole) sample of pentaerythritol arsenite methacrylate and 20 mg. of dicyanobenzoquinone is stirred with 25 ml of acetone and 6 ml of water for 30 minutes at 40°C. The solution is filtered, and the filtrate is stripped to dryness. The residue, in methylene chloride, is dried over calcium sulfate. The solution is again stripped to dryness, and the residue taken up in 8 ml methylene chloride and 8 ml of chlorobenzene. This solution is added to 8.44 g. of ferrocenoyl chloride in 18 ml of chlorobenzene in a flask maintained at 200-mm pressure. When addition is complete, the pressure is reduced to 150 mm and the temperature is maintained at 50°C for 1 hour. The chlorobenzene is removed in vacuo and the residue is partitioned between methylene chloride and water. The organic residue is chromatographed on a silica gel column packed in pentane-methylene chloride (2:1 and 1:1), and methylene chloride gives a center cut of 1.69 g. This portion is re-crystallized from methanol to give pentaerythritol methacrylate tris (ferrocenoate), 1.14g, m.p. 109°-112°C.

Analysis

Calculated for  $C_{42}H_{40}Fe_3O_8$ : C, 60.0; H, 4.80; Fe, 19.94.

Found: C, 59.7; H, 4.80; Fe, 20.9.

**EXAMPLE II**

**Preparation of Pentaerythritol Acrylate tris (ferrocenoate)**

The procedure outlined in Example I above is followed using 1.71 g of pentaerythritol monoacrylate (prepared by hydrolysis of pentaerythritol arsenite acrylate) and 10 g. of ferrocenoyl chloride. The organic residue obtained upon evaporation of the organic sol-

**EXAMPLE III**

**Copolymerization With Butadiene**

Introduce to a glass high-pressure reactor (Aerosol tube): 30 ml. of toluene, 2.112g (0.0084 mole) azo-bis-(2-methyl-5-hydroxy-valeronitrile) as initiator, and 2.1g (0.0025 mole) pentaerythritol methacrylate tris (ferrocenoate). The reactor is attached to a vacuum line and deaerated by three alternate freeze-thaw cycles. Butadiene (10.8g., 0.2 mole) is condensed into the reactor, and the reactor transferred to an oil bath at 66°-67°C. Heating is continued for a period of 72 hours. On cooling the solvent is removed by evaporation and the copolymer reprecipitated by dissolving in ether followed by the addition of methanol. After decanting the solvents, the copolymer is stripped of excess solvents on a rotatory evaporator and finally dried at 70°-75°C. under reduced pressure (1 mm) for a period of 24 hours. The yield of liquid copolymer is 7.1 g (55 percent). The copolymer is characterized by molecular weight (3,500), OH end groups (1.21 wt percent) and elemental analysis (Fe, Found: 3.9).

**EXAMPLE IV**

In a similar reaction to that set forth in Example III, 35 5.4 g. (0.1) butadiene is copolymerized with 2.1g (0.0025 mole) of pentaerythritol methacrylate tris (ferrocenoate) in toluene with 0.756 g. (0.003 mole) azo-bis-(2-methyl-5-hydroxy-valeronitrile) as initiator to give 4.2 g. (56 percent) of the copolymer analyzing 40 as follows: molecular weight (4,700), OH end groups (0.8 weight percent) and elemental analysis (Fe, Found 6.9 percent).

As noted in Examples III and IV the mole ratio of butadiene to monomer is from about 40 to 1 to about 80 45 to 1 for the monomer selected. The mole ratio in Examples III and IV is also satisfactory when the monomer pentaerythritol acrylate tris (ferrocenoate) is selected for copolymer preparation.

**Burning Rate Data**

The hydroxy-terminated copolymer of butadiene and

60 pentaerythritol methacrylate tris-(ferrocenoate) containing 3.9 percent Fe, (prepolymer A of Table I), provides a significant increase in propellant burning rate. Table I below summarizes the data as compared with the standards set forth therein.

65 Similarly, the hydroxy-terminated copolymer of butadiene and pentaerythritol acrylate tris (ferrocenoate) may be used in place of the prepolymer, butadiene and pentaerythritol methacrylate tris (ferrocenoate).

Table I

| Prepolymer % | Plasticizer % | Burning Rates of Uncured Composite Propellants |      |            |      | $R_b$ at 750 psi | $R_b$ at 1500 psi |
|--------------|---------------|------------------------------------------------|------|------------|------|------------------|-------------------|
|              |               | NH <sub>4</sub> ClO <sub>4</sub> %             | Al % | Additive % |      |                  |                   |
| HTPB* 10     | Isodecyl      | 70                                             | 10   | —          | 0.54 | 0.84             |                   |
|              | Pelargonate   | 70                                             | 10   | —          | 0.71 | 0.97             |                   |
| A            | Isodecyl      | 70                                             | 10   | —          | 0.71 | 0.97             |                   |
|              | Pelargonate   | 70                                             | 10   | NBF**, 2   | 0.71 | 0.97             |                   |
| HTPB* 8      | Isodecyl      | 70                                             | 10   | NBF**, 2   | 0.71 | 0.97             |                   |
|              | Pelargonate   |                                                |      |            |      |                  |                   |

\*Unmodified hydroxy-terminated polybutadiene.

\*\*n-butyl ferrocene, a standard burning-rate promoter.

Isodecyl pelargonate is available under the trademark, Emolein from Emery Industries, Inc. Other suitable plasticizers include diisooctyl azelate, di-2-ethylhexyl azelate, and dipropylene glycol diperlargonate.

The plasticizers noted above may be used with the copolymers of this invention in amounts from about 5 to about 25 weight percent of the propellant composition. The ammonium perchlorate may vary from about 50 to about 70 weight percent of the propellant composition. The copolymers of this invention may be used in propellant compositions in amounts from about 5 to about 30 weight percent. Aluminum metal from about 5 to about 20 weight percent may be used in the propellant composition containing the copolymers of this invention.

The copolymers of this invention may be substituted for polybutadiene and the burning rate catalyst employed in a propellant composition since the copolymers contain a catalyst as an integral part thereof. The copolymers of this invention are particularly attractive as a source of catalysis for the propellant composition in order to avoid the problems associated with the use of liquid catalysts (e.g. problems, such as, loss by evaporation or migration within the propellant during storage).

We claim:

1. A propellant composition comprising ammonium perchlorate in an amount from about 50 to about 70 weight percent; aluminum metal in an amount from about 5 to about 20 weight percent; a plasticizer se-

lected from diisooctyl azelate, di-2-ethylhexyl azelate, dipropylene glycol dipelargonate, and isodecyl pelargonate in an amount from about 5 to about 25 weight percent of the propellant composition; and copolymers in an amount from about 5 to about 30 weight percent, said copolymers being formed from butadiene reacted with a polymerizable monomer selected from pentaerythritol metacrylate tris(ferrocenoate) and pentaerythritol acrylate tris(ferrocenoate), said butadiene and said monomer being reacted in a mole ratio of butadiene to monomer from about 40 to 1 to about 80 to 1 while in the presence of a suitable initiator contained in a suitable organic solvent for a predetermined period of time and at a predetermined temperature to form said copolymers; said suitable initiator being azo-bis-(2-methyl-5-hydroxy-valeronitrile); said suitable organic solvent being toluene; said predetermined period of time being about 72 hours; said predetermined temperature being from about 66°C to about 67°C; said copolymers being characterized by a molecular weight in the range from about 3,500 to about 4,700, OH end groups from about 0.8 to 1.2 weight percent, and Fe content from about 3.9 to about 6.9 weight percent.

2. The propellant composition of claim 1 wherein said plasticizer is isodecyl pelargonate present in an amount of about 10 weight percent, said ammonium perchlorate is present in an amount of about 70 weight percent, said copolymers are present in an amount of about 10 weight percent, and aluminum metal is present in an amount of about 10 weight percent.

\* \* \* \* \*

45

50

55

60

65